



US006862418B2

(12) **United States Patent**  
Morita et al.

(10) **Patent No.:** **US 6,862,418 B2**  
(45) **Date of Patent:** **Mar. 1, 2005**

(54) **COLOR IMAGE FORMING APPARATUS**

(75) Inventors: **Kazushige Morita**, Nara (JP); **Yuriko Shindoh**, Yamatokoriyama (JP); **Hiroko Ishibashi**, Ikoma (JP); **Yoshihide Shimoda**, Nara (JP); **Masanori Matsumoto**, Kashihara (JP)

(73) Assignee: **Sharp Kabushiki Kaisha**, Osaka (JP)

(\*) Notice: Subject to any disclaimer, the term of this patent is extended or adjusted under 35 U.S.C. 154(b) by 5 days.

(21) Appl. No.: **10/387,537**

(22) Filed: **Mar. 14, 2003**

(65) **Prior Publication Data**

US 2003/0206754 A1 Nov. 6, 2003

(30) **Foreign Application Priority Data**

Mar. 15, 2002 (JP) ..... 2002-072179

(51) **Int. Cl.** **7 G03G 15/01**

(52) **U.S. Cl.** **399/223; 399/299; 430/46**

(58) **Field of Search** **..... 430/46; 399/299, 399/223, 303**

(56) **References Cited**

**U.S. PATENT DOCUMENTS**

5,202,727 A \* 4/1993 Izumizaki et al. ..... 399/82  
6,403,270 B2 \* 6/2002 Itami et al. ..... 430/59.5

**FOREIGN PATENT DOCUMENTS**

JP 11-024358 A 1/1999  
JP 11-052599 A 2/1999

|    |               |         |
|----|---------------|---------|
| JP | 10-333393 A   | 12/1999 |
| JP | 2000-242056 A | 9/2000  |
| JP | 2000-242057 A | 9/2000  |
| JP | 2000-330303 A | 11/2000 |
| JP | 2001-051467 A | 2/2001  |
| JP | 2001-249576 A | 9/2001  |

\* cited by examiner

*Primary Examiner*—John L. Goodrow

(74) *Attorney, Agent, or Firm*—Birch, Stewart, Kolasch & Birch, LLP

(57) **ABSTRACT**

An electrophotographic color image forming apparatus including a multiple number of photoreceptors for multiple development colors including black, is constructed such that the photoreceptors satisfy the following relation:

$$0.5 < (X/Y) < 0.8,$$

where X represents the reduction in film thickness ( $\text{\AA}$ ) per  $1 \times 10^7$  mm of the traveling distance of the photoreceptor for black development and Y represents the reduction in film thickness ( $\text{\AA}$ ) per  $1 \times 10^7$  mm of the traveling distance of the photoreceptors for the other development colors. This limitation is aimed at differentiating the abrasion resistance of the photoreceptors between that for black and that for colors and designating the reduced amounts of the film thickness per unit traveling distance to fall within the predetermined ranges, whereby it is possible to prevent the drum for black development, which is used most frequently, alone, from being worn away at an earlier time. Accordingly, both the drums for black and for colors can be replaced at approximately the same time, to the maintenance cost can be reduced.

**12 Claims, 3 Drawing Sheets**

FIG. 1



FIG. 3



FIG. 2



FIG. 4



## COLOR IMAGE FORMING APPARATUS

## BACKGROUND OF THE INVENTION

## (1) Field of the Invention

The present invention relates to a color image forming apparatus such as a color printer, etc., and relates to a so-called tandem type color image forming apparatus wherein a multiple number of photoreceptors are charged so as to develop color images by developing devices holding different color toners.

## (2) Description of the Prior Art

Recently, in the field of color electrophotographic processing, tandem type color image forming apparatuses in which a multiple number of photoreceptor drums for multiple colors of toner are arranged in line to obtain a color image have been used in order to enhance the printing speed. This tandem type configuration lends itself to color image forming apparatuses and multi-color image forming apparatuses for outputting image formed articles of reproduction and composition of color images and multi-color images by successively transferring a plurality of color separation images for color image data or multi-color image data, in a layered manner, as well as image forming apparatuses including a color image forming function or multi-color image forming function. It is essential for these image forming apparatuses that all the photoreceptors arranged therein should always have the same level of quality in order to provide images without color imbalance between the color components.

Even if uniform images free from unevenness can be obtained when all the photoreceptors are unused, the problem may take place that the image quality becomes degraded as the photoreceptors are worn down as they are used. Despite of its name, a color image forming apparatus in practice is often used for monochrome (black/white) printing other than color printing. There are cases where monochrome printing is implemented more often than color printing, hence there is a drawback that the photoreceptor for black images becomes worn away earlier than the other color photoreceptors.

Usually, the processing system is designed so that the four photoreceptors for the four colors Y, M, C and K(Bk) toners will not present inharmonious wear characteristics. If, however, the photoreceptors for individual toners are worn away in different manners, there occurs color unevenness and color imbalance as the number of copies increases. In such cases, all the drums, instead of the drum which, alone, has been heavily degraded, should be replaced. Particularly, if hard papers such as post cards are used, large wear takes place locally, causing large influences.

Further, when contact type chargers which will impose heavier burdens on the photoreceptors are used, the amounts of wear of the drums become large. If the wear of the photoreceptor is made small and uniform, it is possible to make the interval for replacement of the drum longer. Further, if all the drums reach the end of their life at almost the same time, concurrent replacement of all the drums will never produce any loss. However, if the wear and degradation rates of the drums differ between different colors of developing devices, degradation of only one of them requires replacement of all the drums. Otherwise, color imbalance between the new drum and the other drums, which have not been replaced, takes place, resulting in failure to obtain good image quality. In other words, the interval of drum replacement is determined by the most intensively degraded drum among the four. This results in being wasteful and uneconomical.

As countermeasures, Japanese Patent Application Laid-open Hei 10 No.333393, Japanese Patent Application Laid-

open Hei 11 No.24358 and Japanese Patent Application Laid-open Hei 11 No. 52599, disclose configurations in which an  $\alpha$ -Si or  $\alpha$ -SiC photoreceptor is used for that for black development so as to enhance the photoreceptor life while OPCs (organic photoreceptors) are used for those other than that for black development. There is, however, a problem that  $\alpha$ -Si and  $\alpha$ -SiC photoreceptors used in the above publications are less chargeable. As a solution to this drawback, Japanese Patent Application Laid-open Hei 10 No.333393 specifies the thickness of the photoreceptor to be 30  $\mu$ m or more and its difference in surface potential from the other organic photoreceptors to be equal to or lower than 200 V. Japanese Patent Application Laid-open Hei 11 No.24358 proposes that the applied voltage to the  $\alpha$ -Si photoreceptor should be 1.05 to 2.50 times the application voltage to the organic photoreceptors. Further, Japanese Patent Application Laid-open Hei 11 No.52599 is aimed at increasing the chargeability by adding an  $\alpha$ -SiC surface layer.

In the above way, in order to extend the life of the photoreceptor for black development while making up for the low chargeability of the  $\alpha$ -Si or  $\alpha$ -SiC photoreceptor, it is necessary to make complicated charge control for black development, resulting in the need of extra cost. Further, since, other than the charge control, there are differences in light sensitivity and susceptibility to temperature/humidity, between the  $\alpha$ -Si or  $\alpha$ -SiC photoreceptor and the organic photoreceptor, light exposure, transfer conditions and other factors differ between the  $\alpha$ -Si or  $\alpha$ -SiC photoreceptor for black development and the organic photoreceptors for development other than black. Therefore, a different control method of the photoreceptor for black development from that for the photoreceptors for the other colors should be used, thus again resulting in the need of extra cost. The  $\alpha$ -Si or  $\alpha$ -SiC photoreceptors disclosed in Japanese Patent Application Laid-open Hei 10 No.333393, Japanese Patent Application Laid-open Hei 11 No.24358 and Japanese Patent Application Laid-open Hei 11 No.52599, have the problem that their production cost is obviously high compared to the organic photoreceptors. Further, as another problem, they consume large amounts of black toner, as is well known.

As the countermeasures against the above problems, Japanese Patent Application Laid-open 2000 Nos.242056 and 242057 propose configurations where the drum for black development alone is increased in diameter or increased in film thickness. Japanese Patent Application Laid-open 2001 No.51467 refers to use of a non-contact type charging means only for black development, increase in film thickness and use of a resin having a large viscosity-average molecular weight. Further Japanese Patent Application Laid-open 2000 No.330303 discloses a polycarbonate copolymer resin as the resin for tandem photoreceptors. Further, provision of a protective layer on only the photoreceptor for black development has been also investigated as an optional method.

Increase of the drum diameter for black development alone as in Japanese Patent Application Laid-open 2000 Nos.242056 and 242057 results in enlargement of the machine body. Increase in thickness of the coating film may cause reduction in the amount of charge or degrade dot reproducibility and/or line reproducibility in the image. Further, use of a resin having a large viscosity-average molecular weight produces an air entrapment problem when it is applied and causes difficulties in application. Japanese Patent Application Laid-open 2000 No.330303 also discloses use of various copolymer polycarbonate resins as the resin for tandem photoreceptors and refers to the relationship between the maximum/minimum abrasion losses. However, the discussed photoreceptors for black and other color development use an identical configuration, hence it is

impossible to lengthen the life of the photoreceptor for black development in a general environment in which monochrome copy mode is used often.

On the other hand, Japanese Patent Application Laid-open 2001 No.249576 refers to increase in film thickness of the photoreceptor layer in order to improve the abrasion resistance of the photoreceptive layer of the photoreceptor used in the image forming and transfer unit undergoing a greater contact abrasive force. However, when, for example, a silicon photoreceptor presenting a markedly large abrasion resistance is used for black development only, the photoreceptor for black images, alone, is still usable despite the photoreceptors for colors having already reached the end of their life, bringing about a reversal in the relationship, so this cannot be said to be the perfect solution.

### SUMMARY OF THE INVENTION

The present invention is aimed at solving the above conventional problems and attaining the following object. It is therefore an object of the present invention to provide a color image forming apparatus in which all the photoreceptors, even though use frequencies are different across the colors, may have approximately the same life and which is low in maintenance cost.

A color image forming apparatus of the present invention comprises a multiple number of electrophotographic image forming stations for multiple development colors including black, arranged in line in the paper feed direction, each image forming station having a photoreceptor, a charger, an exposure device, a developing device, a transfer device and a cleaning device, and is characterized in that the photoreceptors satisfy the following relation:

$$0.5 < (X/Y) < 0.8,$$

where X represents the reduction in film thickness (Å) per  $1 \times 10^7$  mm of the traveling distance of the photoreceptor for black development and Y represents the reduction in film thickness (Å) per  $1 \times 10^7$  mm of the traveling distance of the photoreceptors for the other development colors.

In this case, it is possible to lengthen the life of the photoreceptor for black development, which is used most frequently, compared to the life of the photoreceptors used for the other development colors, conforming to the empirically acquired usage frequencies of all the colors. Accordingly, it is possible to prevent the drum for black development, which is used most frequently, alone, from reaching the end of life at an earlier time, so that both the drum for black and the drums for colors can be replaced at approximately the same time.

The present invention is also characterized in that the binder resin used for either the photoreceptor for black development or at least one of the photoreceptors for the other development colors employs a polycarbonate polymer having, at least, one structural unit represented by the following general formula (1):

(1)



(wherein R<sup>1</sup>, R<sup>2</sup>, R<sup>3</sup>, R<sup>4</sup>, R<sup>5</sup>, R<sup>6</sup>, R<sup>7</sup> and R<sup>8</sup> individually represent a hydrogen atom, halogen atom, substituted or

unsubstituted alkyl of 1 to 6 carbon atoms, C<sub>4</sub>-C<sub>10</sub> cyclic hydrocarbon residual group, substituted or unsubstituted aryl, and Z represents a group of atoms required to constitute a substituted or unsubstituted cycle or substituted or unsubstituted hetero-cycle, m being an integer).

Accordingly, when the present invention is realized, it is possible to improve and control the image stability against ozone, NO<sub>x</sub> and the like and enhance the plate wear.

The present invention is also characterized in that the binder resin used for either the photoreceptor for black development or the photoreceptors for the other development colors employs a polycarbonate polymer having, at least, one structural unit represented by the general formula (1).

Accordingly, when the present invention is realized, it is possible to improve the image stability against ozone, NO<sub>x</sub> and the like and enhance the plate wear.

The image forming apparatus of the present invention is also characterized in that the photoreceptors other than that for black development are stopped operating in monochrome (black and white) copy mode.

Accordingly, rotation of the unnecessary photoreceptors can be obviated so that it is possible to reduce the film abrasion of the photoreceptors other than that for black development.

The image forming apparatus of the present invention is further characterized in that the photoreceptors other than that for black development are separated from the recording media conveyer belt, in monochrome (black and white) copy mode.

Accordingly, since the photoreceptors other than that for black development are separated from the recording media conveyer belt, in monochrome (black and white) copy mode, it is possible to avoid the chance of the coating films of the photoreceptors being abraded by recording media and/or the recording media conveyer belt or the like, hence lengthen the life of the photoreceptors.

The image forming apparatus of the present invention is characterized in that the film thickness of the photoreceptor layer ranges from 18  $\mu\text{m}$  to 27  $\mu\text{m}$ .

In this case, it is possible to produce good images without any loss of dot reproducibility or line reproducibility in the images.

As to the shape and/or appearance of the photoreceptors or their parts in the image forming apparatus, the shape and/or appearance of the photoreceptor for black development or its part is made different from the shape and/or appearance of the photoreceptors or their parts for the other development colors.

There are cases where the photoreceptors of different colors cannot be differentiated only from their appearances. Designing them so as to be incompatible to each other obviates misplacement of the photoreceptors into the wrong places, hence intended result can be positively be achieved.

### BRIEF DESCRIPTION OF THE DRAWINGS

FIG. 1 is a schematic sectional view of a layered photoreceptor according to the embodiment of the present invention;

FIG. 2 is a schematic front sectional view showing the configuration of a digital color copier as an image forming apparatus of the present invention;

FIG. 3 is a flowchart showing the operational control in accordance with the output image mode designation; and

FIG. 4 is a CuK $\alpha$  characteristic X-ray diffraction chart of an oxotitanyl phthalocyanine pigment used in the embodiment of the present invention.

### DESCRIPTION OF THE PREFERRED EMBODIMENTS

The embodiment of the present invention will hereinafter be described in detail with reference to the accompanying drawings.

To begin with, the constituent materials in the schematic sectional view of a layered photoreceptor shown in FIG. 1 as one embodiment of the photoreceptor of the present invention will be described. In FIG. 1, 1 designates a conductive substrate, 2 a charge generation layer, 3 a charge transport layer, 4 a photosensitive layer of the photoreceptor consisting of an undercoat layer, charge generation layer and charge transport layer, and 5 an undercoat layer provided between the conductive substrate and the charge generation layer.

As conductive substrate 1, metals such as aluminum, copper, brass, zinc, nickel, stainless steel, chromium, molybdenum, vanadium, indium, titanium, gold and platinum and alloys of these can be used. Other than these, polyester film, paper and metal film on which aluminum, aluminum alloy, tin oxide, gold, indium oxide or the like is deposited or applied, plastic and paper containing conductive particles, and plastics containing conductive polymers or the like can be used. These materials are shaped and used in a cylindrical, columnar form or in a film sheet form.

Undercoat layer (intermediate layer) 5 may be provided between conductive substrate 1 and charge generation layer 2. As the undercoat layer 5, an inorganic layer such as an anodic oxide thin film formed on aluminum, aluminum oxide, aluminum hydroxide and the like, an organic layer such as polyvinyl alcohol, casein, polyvinyl pyrrolidone, polyacrylic acid, celluloses, gelatin, starch, polyurethane, polyimide, polyamide and the like and an organic layer containing as inorganic pigments, conductive or semiconductive particles, of metal such as aluminum, copper, tin, zinc, titanium or the like or of metal oxide such as zinc oxide, aluminum oxide, titanium oxide or the like, can be used. As to crystalline types of titanium oxide, there are various types such as the anatase form, rutile form and amorphous type, and any of these can be used alone or in combination. Titanium oxide particles covered with  $\text{Al}_2\text{O}_3$ ,  $\text{ZrO}_2$  or the like or a combination of these can be preferably used.

As the binder resin contained in undercoat layer 5, polyvinyl alcohol, casein, polyvinyl pyrrolidone, polyacrylic acid, celluloses, gelatin, starch, polyurethane, polyimide, polyamide and other resins can be used. Among these, polyimide resin is preferably used. This is because the binder resin of the undercoat layer is demanded to be insoluble and non-swelling in the solvent used for forming the photoconductive layers over undercoat layer 5, and to present excellent adhesiveness to conductive substrate 1 and enough flexibility. Among polyimide resins, alcohol-soluble nylon resins can be more preferably used. Specific examples of the resin include so-called copolymer nylons having 6-nylon, 66-nylon, 610-nylon, 11-nylon, 12-nylon and others compolymerized, and chemically modified nylons such as N-alkoxymethyl denatured nylon.

In the present invention, general solvents can be used as the organic solvent for the application liquid of undercoat layer 5, but it is preferred that, when alcohol-soluble nylon resin, which is more preferable, is used as the binder resin, a pure or mixture type organic solvent selected from the lower alcohol group having 1 to 4 carbon atoms and another group of organic solvents including dichloromethane, chloroform, 1,2-dichloroethane, 1,2-dichloropropane, toluene, tetrahydrofuran and 1,3-dioxolane be preferably used. In this case, mixing the pure alcohol solvent with the above organic solvent improves dispersibility of titanium oxide in the solvent compared to that in the pure alcohol solvent, so that it is possible to make the stability under storage long-lasting and reuse the application liquid. This also prevents coating defects and uneven coating of undercoating layer 5 when the conductive substrate is dip coated in the application liquid for undercoat layers to form under-

coat layer 5, whereby it is possible to achieve uniform application of the photoconductive layer thereon, which leads to provision of an electrophotographic photoreceptor excellent in imaging characteristics and free from film defects.

Production of undercoat layer 5 can be carried out using an undercoat layer application liquid that has been prepared by blending the above inorganic pigment with a solvent and binder resin and dispersing the mixture by means of a ball mill, Dyno-mill, supersonic oscillator or other dispersing machines. For a sheet-like substrate, a baker applicator, bar coater, casting, spin coating or other methods can be used. For a drum substrate, a spray method, vertical ring method, dip coating or other methods can be used.

Charge generation layer 2 is mainly composed of a charge generating material which generates electric charges by illumination of light, and contains publicly known binder, plasticizer and sensitizer, as necessary. Examples of the charge generation material include: perylene pigments such as peryleneimide, perylenic anhydride; polycyclic quinone pigments such as quinacridone, anthraquinone; phthalocyanine pigments such as metal and metal-free phthalocyanines, halogenated metal-free phthalocyanine; squarium dyes; azuleneum dyes; thiapyrillium dyes; and azo pigments having a carbazole skeleton, styryl stilbene skeleton, triphenylamine skeleton, dibenzothiophene skeleton, oxadiazole skeleton, fluorenone skeleton, bis-stilbene skeleton, distyryl oxadiazole skeleton or distyryl carbazole skeleton.

In particular, metal-free phthalocyanine pigments, oxotitananyl phthalocyanine pigments, bisazo pigments containing a fluoren ring or fluorenone ring, bisazo pigments consisting of aromatic amines and triazo pigments can present especially high charge generation power, so that use of these provides a high sensitive photoreceptor. Further, with concern to oxotitananyl phthalocyanines, a crystalline type which presents a diffraction peak at a Bragg angle ( $2\theta \pm 0.2^\circ$ ) of  $27.3^\circ$  in the X-ray diffraction spectrum can provide a further high sensitivity and so is more preferred.

Production of charge generation layer 2 can be carried out using an application liquid that has been prepared by blending the fine particles of the above charge generation material with an organic solvent and pluverizing and dispersing the particles by means of a ball mill, sand grinder, paint shaker, supersonic dispersing machine or the like. For a sheet-like substrate, a baker applicator, bar coater, casting, spin coating or other methods can be used. For a drum substrate, a spray method, vertical ring method, dip coating or other methods can be used.

In order to enhance the binding property, binder resins as follows may be added, for example: polyester resin, polyvinyl acetate, polyacrylic ester, polycarbonate, polyacrylate, polyvinyl acetoacetal, polyvinyl propynal, polyvinyl butyral, phenoxy resin, epoxy resin, urethane resin, melamineresin, siliconeresin, acrylicresin, celluloseester, cellulose ether, vinylchloride-vinyl acetate copolymer resin. The film thickness is preferably 0.05 to 5  $\mu\text{m}$ , more preferably 0.1 to 1  $\mu\text{m}$ . The charge generation layer may contain various additives such as a leveling agent for improving application performance, antioxidant and sensitizer, as required.

Charge transport layer 3 provided over charge generation layer 2 essentially consists of a charge transport material for accepting charges generated within the charge generation material, and transporting them, and a binder (binder resin). As the charge transport material, the following electron donative materials can be used: poly-N-vinyl carbazole and its derivatives, poly-g-carbazolyl ethylglutamate and its derivatives, pyrene-formaldehyde condensate and its derivatives, polyvinyl pyrene, polyvinyl phenanthrene, oxazole derivatives, oxadiazole derivatives, imidazole

derivatives, 9-(*p*-diethylamine styryl) anthracene, 1,1-bis (4-dibenzyl aminophenyl) propane, styryl anthracene, styryl pyrazoline, pyrazoline derivatives, phenylhydrazones, hydrazone derivatives, triphenylamine compounds, tetraphenyl diamine compounds, triphenylmethane compounds, stilbene compounds, azine compounds having a 3-methyl-2-benzothiazoline ring, etc.

Alternatively, the following electron acceptable substances can be used: fluorenone derivatives, dibenzothiophene derivatives, indeno thiophene derivatives, phenanthrene quinone derivatives, indeno pyridine derivatives, thioxanthone derivatives, benzo[c]cinnoline derivatives, phenazine oxide derivatives, tetracyanoethylene, tetracyanoquinodimethane, bromanil, chloranil, benzoquinone, etc. Of these, particular types of butadiene compounds, styryl compounds and amine compounds, having the following structure are more preferable in the present invention since they show high hole transporting properties so that a high sensitivity can be maintained even when the resin ratio is high. One example is shown below.



(wherein  $\text{Ar}_1$ ,  $\text{Ar}_2$ ,  $\text{Ar}_3$  and  $\text{Ar}_4$  each represent an aryl which may have a substituent, at least one of  $\text{Ar}_1$  to  $\text{Ar}_4$  being an aryl having an amino-substituent as its substituent and  $n$  being 0 or 1.)

As the specific examples of the general formula (2), the following compounds (2-1) to (2-12) can be mentioned.



-continued



20

**9**

-continued

**10**

(3-1)



(3)



As styryl compounds, the compounds having the following general form (3) can be mentioned. 50  
(wherein Ar<sub>5</sub> represents an aryl which may have a substituent, Ar<sub>6</sub> represents a phenylene, naphthylene, biphenylene or anthrylene which may have a substituent, R<sup>9</sup> represents a hydrogen atom or lower alkyl or lower alkoxy, X represents a hydrogen atom or an alkyl which may have a substituent, or an aryl which may have a substituent, and Y represents an aryl which may have a substituent). 60 65

As the specific examples of the general formula (3), the following compounds (3-1) to (3-16) can be mentioned. 65



**11**

-continued

**12**

-continued



(3-7)



(3-8)



(3-9)



(3-10)



(3-13)



(3-14)



(3-15)



**13**  
-continued

(3-16)



As amine compounds, the compounds having the following general formula (4) can be mentioned.

(4)



(wherein R<sub>10</sub> to R<sub>15</sub> each represent a hydrogen atom, halogen atom, alkyl, alkoxy, p, q, r, s, t and u indicating an integer 1 to 5).

As specific examples of the general formula (4), the following compounds (4-1) to (4-6) can be mentioned.

(4-1)



40

45

(4-2)



50

55

(4-3)



60

65

**14**  
-continued

(4-4)



(4-5)



(4-6)



Generally, the binder resin is selected from those which are compatible with the charge transport material. Examples include vinyl polymers such as polymethylmethacrylate, polystyrene and polyvinyl chloride, polycarbonate resin, polyester resin, polyester carbonate resin, polysulfone resin, phenoxyresin, epoxyresin, silicone resin, polyacrylates resin, polyimide resin, polyurethane resin, polyacrylamide resin and phenol resin.

These resins can be used alone or in combination, or may be partially cross-linked so to present thermosetting properties. In particular, polystyrene, polycarbonate, polyacrylate and polyphenylene oxide resins have a volume resistivity of 10<sup>13</sup> Ω or greater and are excellent in coating performance and electric characteristics.

As the binder resin used here, polycarbonate polymers having repeat units of the following general form (5) are preferably used.

(5)



(wherein each R<sup>2'</sup> individually represents a halogen atom, vinyl, allyl, substituted or unsubstituted alkyl of 1 to 10 carbon atoms, substituted or unsubstituted aryl of 6 to 12 carbon atoms, substituted or unsubstituted cycloalkyl of 3 to 12 carbon atoms, substituted or unsubstituted alkoxy of 1 to 6 carbon atoms, or substituted or unsubstituted aryloxy of

## 15

6 to 12 carbon atoms, 'a' being an independent integer of 0 to 4, Y representing single bond, —O—, —CO—, —S—, —SO—, SO<sub>2</sub>—, —CR<sup>3</sup>R<sup>4</sup>—, substituted or unsubstituted cycloalkylidene of 5 to 11 carbon atoms, substituted or unsubstituted a,  $\omega$ -alkylene of 2 to 12 carbon atoms, 9,9-fluorenylidene, 1,8-menthane diyl, 2,8-menthane diyl, substituted or unsubstituted pyrazilidene, or substituted or unsubstituted arylene of 6 to 24 carbon atoms. Here, R<sup>3</sup> and R<sup>4</sup> individually represent a hydrogen atom, or substituted or unsubstituted alkyl of 1 to 10 carbon atoms, or substituted or unsubstituted aryl of 6 to 12 carbon atoms.)

The polycarbonate polymer used in the present invention may have one or more types of repeat units having the general form (5). Further, the polycarbonate polymer may contain repeat units other than that having the general form (5), as long as no obstruction to the achievement of the object of the present invention occurs.

In the general representation (5), specific examples of R<sup>2</sup>, Y, R<sup>3</sup> and R<sup>4</sup> are as follows.

Examples of a halogen atom represented by R<sup>2</sup> include fluorine, chlorine, bromine and iodine. Of these, fluorine, chlorine and bromine are preferred.

Examples of the unsubstituted alkyl of 1 to 10 carbon atoms, represented by R<sup>2</sup>, R<sup>3</sup> and R<sup>4</sup>, include methyl, ethyl, propyl, isopropyl, butyl, 2-butyl, tert-butyl, isobutyl, pentyl, hexyl, heptyl, octyl, nonyl and decyl. Of these, methyl, ethyl, propyl, isopropyl, butyl, 2-butyl and tert-butyl are preferred.

Examples of the unsubstituted aryl of 6 to 12 carbon atoms, represented by R<sup>2</sup>, R<sup>3</sup> and R<sup>4</sup>, include phenyl, naphthyl and biphenyl, and phenyl is preferred. Examples of the unsubstituted cycloalkyl of 3 to 12 carbon atoms, represented by R<sup>2</sup>, include cyclopentyl, cyclohexyl and cycloheptyl. Of these cyclopentyl and cyclohexyl are preferred.

Examples of the unsubstituted alkoxy of 1 to 6 carbon atoms, represented by R<sup>2</sup>, include methyl oxyl, ethyl oxyl, propyl oxyl, isopropyl oxyl, butyl oxyl, 2-butyl oxyl, tert-butyl oxyl, isobutyl oxyl, pentyl oxyl and hexyl oxyl. Of these, methyl oxyl, ethyl oxyl, propyl oxyl and isopropyl oxyl are preferred.

Examples of the unsubstituted aryloxy of 6 to 12 carbon atoms, represented by R<sup>2</sup>, include phenyl oxyl, naphthyl oxyl and biphenyl oxyl. Of these, phenyl oxyl is preferred. Examples of the unsubstituted arylene of 6 to 24 carbon atoms, represented by Y, include phenylene, naphthylene, biphenylylene, terphenylylene and quaterphenylylene. Of these, phenylene is preferred.

Examples of the unsubstituted cycloalkylidene of 5 to 11 carbon atoms, represented by Y, include cyclopentylidene, cyclohexylidene, cycloheptylidene, cyclooctylidene, cyclononylidene, cyclodecylidene and cycloundecylidene. Of these, cyclohexylidene is preferred.

Examples of the unsubstituted  $\alpha$ ,  $\omega$ -alkylene of 2 to 12 carbon atoms, represented by Y, include ethylene, trimethylene, tetramethylene, pentamethylene, hexamethylene, heptamethylene, octamethylene, nonamethylene, decamethylene, undecamethylene and dodecamethylene. Of these, ethylene and trimethylene are preferred. As the 1,8-menthane diyl, represented by Y, 1,8-p-menthane diyl is preferred. As the 2,8-menthane diyl, represented by Y, 2,8-p-menthane diyl is preferred.

The substituted alkyl, substituted aryl, substituted alkoxy, substituted aryloxy, substituted cycloalkyl, substituted arylene, substituted  $\alpha$ ,  $\omega$ -alkylene, substituted cycloalkylidene and substituted pyrazilidene indicate the aforementioned unsubstituted alkyl, unsubstituted aryl, unsubstituted alkoxy, unsubstituted aryloxy, unsubstituted cycloalkyl, unsubstituted arylene, unsubstituted  $\alpha$ ,  $\omega$ -alkylene, unsubstituted cycloalkylidene and unsubstituted

## 16

pyrazilidene, of which one of hydrogen atoms is substituted by a substituent.

Examples of the substituents of the substituted alkyl and substituted alkoxy include halogen atoms (fluorine, chlorine, bromine, iodine), aryls of 6 to 12 carbon atoms (phenyl, naphthyl, biphenyl), alkoxy of 1 to 4 carbon atoms (methoxy, ethoxy, propoxy, isopropoxy, butoxy, sec-butoxy, tert-butoxy, isobutoxy), alkylthiols of 1 to 4 carbon atoms (methylthio, etc.) and arylthiols of 6 to 12 carbon atoms (phenylthio, etc.).

Examples of the substituents of the substituted aryl, substituted aryloxy and substituted arylene include halogen atoms (fluorine, chlorine, bromine, iodine), alkyls of 1 to 4 carbon atoms (methyl, ethyl, propyl, isopropyl, butyl, sec-butyl, tert-butyl, isobutyl), alkoxy of 1 to 4 carbon atoms (methoxy, ethoxy, propoxy, isopropoxy, butoxy, sec-butoxy, tert-butoxy, isobutoxy), alkylthiols of 1 to 4 carbon atoms (methylthio, etc.) and arylthiols of 6 to 12 carbon atoms (phenylthio, etc.).

Examples of the substituents of the substituted  $\alpha$ ,  $\omega$ -alkylene, substituted cycloalkyl, substituted cycloalkylidene and substituted pyrazilidene include halogen atoms (fluorine, chlorine, bromine, iodine), alkyls of 1 to 4 carbon atoms (methyl, ethyl, propyl, isopropyl, butyl, sec-butyl, tert-butyl, isobutyl), aryls of 6 to 12 carbon atoms (phenyl, naphthyl, biphenyl), alkoxy of 1 to 4 carbon atoms (methoxy, ethoxy, propoxy, isopropoxy, butoxy, sec-butoxy, tert-butoxy, isobutoxy), alkylthiols of 1 to 4 carbon atoms (methylthio, etc.) and arylthiols of 6 to 12 carbon atoms (phenylthio, etc.). As a preferred examples of the substituted alkyls of 1 to 10 carbon atoms, substituted by halogen atoms for R<sup>2</sup>, R<sup>3</sup> and R<sup>4</sup>, trifluoromethyl with the three hydrogen atoms of the methyl substituted with fluorine atoms can be mentioned.

When the polycarbonate polymer having the above general form (5) is used alone, the polymer preferably has a viscosity-average molecular weight of 30,000 to 70,000. When it is less than 30,000, the plate wear is markedly reduced. When greater than 70,000, the solution viscosity increases while the plate wear is improved to some degree, hence it takes long time to mix it with the charge transport material and uneven application of coating tends to occur, resulting in a reduced productivity. Use of a polycarbonate polymer having, at least, one structural unit represented by the following general form (1) is especially preferred.



(wherein R<sup>1</sup>, R<sup>2</sup>, R<sup>3</sup>, R<sup>4</sup>, R<sup>5</sup>, R<sup>6</sup>, R<sup>7</sup> and R<sup>8</sup> individually represent a hydrogen atom, halogen atom, substituted or unsubstituted alkyl of 1 to 6 carbon atoms, C<sub>4</sub>—C<sub>10</sub> cyclic hydrocarbon residual group, substituted or unsubstituted aryl. Z represents a group of atoms required to constitute a substituted or unsubstituted cycle or substituted or unsubstituted heterocycle, m being an integer).

As the specific examples of general form (1), the following compounds (1-1) to (1-4) can be mentioned.

17



Since the binder resins represented by the above general formula (1) present low permeability to gas, it is possible to prevent infiltration of gases such as ozone, NO<sub>x</sub> and the like which will degrade photoreceptor characteristics. These resins present excellent compatibility with the charge transport material and also have excellent durability. Blends of these resins also present excellent compatibility with the charge transport material and have excellent durability.

The polycarbonate resin having the above general form (1) preferably has a viscosity-average molecular weight of about 15,000 to 50,000. When it is less than 15,000, while the image stability (image deletion of halftones and occurrence of black stripes) against ozone, NO<sub>x</sub>, etc., generated by the charging process, improves, lowering of the initial sensitivity, increase in remaining potential when used repeatedly and lowering of the image stability become augmented.

Examples of solvents for dissolving these materials include alcohols such as methanol, ethanol, etc., ketones such as acetone, methyl ethyl ketone, cyclohexanone, etc., ethers such as ethylether, tetrahydrofuran, etc., aliphatics such as chloroform, dichloroethane, dichloromethane, etc., halogenated hydrocarbons, aromatics such as benzene, chlorobenzene, toluene, etc.

The ratio between the charge transport material and binder resin is usually set at about 10/15 to 10/6, however, in the present invention, it is preferably set at 10/14 to 10/20, in view of improving abrasion resistance. The application liquid for charge transport layers of the present invention may contain additives such as plasticizer, antioxidant, ultraviolet absorbent, leveling agent and the like, in order to improve film forming performance, flexibility, application performance and the like. When the charge transport substance is contained in a ratio greater than 10/14, good sensitivity is obtained, while the charging characteristics, the mechanical strength of the coating and the image stability (occurrence of image deletion of halftones and black stripes) against ozone, NO<sub>x</sub> and the like, generated during the

18

charging process, degrade. In contrast, when the binder resin is contained in a ratio greater than 10/20, the charging characteristics, the mechanical strength and the image stability are good while the sensitivity markedly lowers. The charge transport layer is preferably formed with a thickness of 15 to 30  $\mu\text{m}$ , more preferably 18 to 27  $\mu\text{m}$ .

In the present invention, the charge transport layer may contain additives such as an antioxidant, leveling agent and the like, together with the above binder resin. As the antioxidant, typical antioxidants which are added to resins can be used as is. For example, vitamin E, hydroquinone, hindered amine, hindered phenol, p-phenylenediamine, arylalkane and their derivatives, organosulfur compounds, organophosphorous compounds and others can be blended. The preferable usage of the antioxidant is 0 to 20 parts by weight relative to 100 parts by weight of the binder resin. As a leveling agent, silicone oils, polymers or oligomers having perfluoroalkyl side chains can be used. The proper usage of the leveling agent is 0 to 1 part by weight relative to 100 parts by weight of the binder resin.

The application liquid for charge transport layers can be prepared without any problem by a typical method in which the charge transport substance, binder resin and additives are measured and then dissolved altogether into a predetermined amount of organic solvent. However, it is preferred that the binder resin has been dissolved first into the solvent and then, the carrier transport substance is added and dissolved therein. This method improves dispersibility of the carrier transport substance in the binder resin and inhibits possible and local crystallization of the carrier transport agent in the film, whereby it is possible to improve the initial sensitivity and potential stability after repeated usage and provide good image characteristics and the like. For application, the same method as used for the undercoat layer and charge generation layer can be used. The proper solvent to dissolve (or disperse) the charge transport substance is, in effect, the same as that used for dispersing the charge generation substance, hence can be selected from the solvents listed for the charge generation material. Among those, tetrahydrofuran is especially preferable.

For attachment of the photoreceptors into a copier or printer, rotational mechanisms are needed. Specifically, a drive transmission part called 'flange' is assembled for each photoreceptor. These flanges usually have the same shape and appearance. In the present invention, the photoreceptor for black development and the photoreceptors for the other development colors or their parts (transmission parts such as flanges, etc.,) should be made different in shape and/or appearance. If their shapes are indistinguishable, the flanges can be made different in color so as to obviate misplacement. Since full performance cannot be obtained if the photoreceptors are set in the wrong places, it is preferred that the flange for the photoreceptor for black should be formed with a different shape from that of the other photoreceptors so it will be incompatible with the others.

Next, the image forming apparatus of the present invention will be described with reference to the accompanying drawing. FIG. 2 is a schematic front sectional view showing the configuration of a digital color copier as an image forming apparatus in accordance with the embodiment of the present invention. The copier body 1 has an original table 111 and a control panel on the top thereof and has an image reading portion 110 and an image forming unit 210 within.

A reversing automatic document feeder (RADF) 112 is arranged on the top surface of original table 111 in a predetermined position with respect to the original table 111 surface whilst being supported so as to be opened and closed relative to original table 111.

RADF 112, first, conveys an original so that one side of the original opposes image reading portion 110 at the predetermined position on original table 111. After the

image scanning of this side is completed, the original is inverted and conveyed to original table 111 so that the other side opposes image reading portion 110 at the predetermined position on original table 111. Then, when RADF 112 completes image scanning of both sides of one original, the original is discharged and the duplex copy conveying operation for a next document is implemented. The operation of the conveyance and face inversion of the original is controlled in association with the whole copier operation.

Image reading portion 110 is disposed below original table 111 in order to read the image of the original conveyed onto original table 111 by means of RADF 112. Image reading portion 110 includes original scanning portion 113 and 114 which reciprocates along, and in parallel to, the undersurface of original table 111, an optical lens 115 and a CCD line sensor 116 as a photoelectric converting device. This original scanning portion 113 and 114 is composed of first and second scanner units 113 and 114. First scanner unit 113 has an exposure lamp for illuminating the original image surface and a first mirror for deflecting the reflection image of light from the original toward the predetermined direction and moves at the predetermined speed in a reciprocating manner in parallel with, whilst being kept a certain distance away from, the undersurface of original table 111.

Second scanner unit 114 has second and third mirrors which deflect the reflected light image from the original, deflected by first mirror of first scanner unit 113 toward the predetermined direction and moves in a reciprocating manner at a speed related to that of first scanner unit 113 and in parallel thereto. Optical lens 115 reduces the reflected light image from the original, thus deflected by third mirror of the second scanner unit, so that the reduced light image will be focused on the predetermined position on CCD line sensor 116.

CCD line sensor 116 implements sequential photoelectric conversion of the focused light image into electric signals and outputs them. CCD line sensor 116 is a three-line color CCD which reads monochrome or color images and outputs line data as to color separation components R(red), G(green) and B(blue). The original image information thus obtained in the electric signal form from this CCD line sensor 116 is further transferred to an after mentioned image processor where predetermined image data processes are performed.

Next, the configuration of image forming unit 210 and the configuration of the components related to image forming unit 210 will be described. Provided below image forming unit 210 is a paper feeding mechanism 211 which separates a sheet of paper (recording medium) P, one by one, from a stack of paper held in a paper tray and feeds it toward image forming unit 210. The paper P thus separated is delivered into image forming unit 210 with its timing controlled by a pair of registration rollers 212 located before image forming unit 210. The paper P with an image formed on its one side is conveyed and re-fed to image forming unit 210 in time with image forming of image forming unit 210.

Arranged under image forming unit 210 is a conveyer and transfer belt mechanism 213. A conveyer and transfer belt 216 of conveyer and transfer belt mechanism 213 is wound and tensioned between a driving roller 214 and an idle roller 215 so that the upper and lower parts of the belt extend approximately parallel to each other. The conveyer and transfer belt 216 electrostatically attracts paper P to itself to convey it. Further, a pattern image detecting unit is provided under and in proximity to conveyer and transfer belt 216. Arranged in the paper conveyance path, downstream of conveyer and transfer belt mechanism 213 is a fixing unit 217. This fixing unit 217 fixes the transferred toner image onto paper P. The paper P having passed through the nip between a pair of fixing rollers of fixing unit 217 passes through a conveyance direction switching gate 218 and is discharged by discharge rollers 219 to a paper output tray 220 attached to the outer wall of copier body 1.

This switching gate 218 selectively connects the conveyance path of paper P after fixing with either the path to discharge paper P to the outside of copier body 1 or the path to recirculate paper P toward image forming unit 210. The paper P which is designated to be conveyed again to image forming unit 210 by means of switching gate 218 is inverted by means of a switch-back conveyance path 221 and then re-fed to image forming unit 210.

Arranged above, and in proximity to, conveyer and transfer belt 216 in image forming unit 210 are the first image forming station Pa, the second image forming station Pb, the third image forming station Pc and the fourth image forming station Pd, in the above mentioned order from the upstream side of the paper conveyance path.

Conveyer and transfer belt 216 is frictionally driven by driving roller 214 in the direction indicated by arrow Z in FIG. 2, and carries paper P which is fed by paper feeding mechanism 211 as stated above and sequentially conveys it through image forming stations Pa to Pd.

All the image forming stations Pa to Pd are of a substantially identical configuration. Each image forming station Pa, Pb, Pc and Pd has a photoreceptor drum 222a, 222b, 222c and 222d, which is driven in the rotational direction indicated by arrow F in FIG. 2. Provided around each photoreceptor drum 222a-222d, are a primary charger 223a, 223b, 223c and 223d for uniformly charging photoreceptor drum 222a-222d, a developing unit 224a, 224b, 224c and 224d for developing the static latent image formed on photoreceptor drum 222a-222d, a transfer charger 225a, 225b, 225c and 225d for transferring the developed toner image on photoreceptor drum 222a-222d to paper P, and a cleaning unit 226a, 226b, 226c and 226d for removing the leftover toner from photoreceptor drum 222a-222d, in this order with respect to the rotational direction of each photoreceptor drum 222a-222d.

Arranged above photoreceptor drums 222a-222d are laser beam scanner units 227a, 227b, 227c and 227d, respectively. Each laser beam scanner unit 227a-227d includes: a semiconductor laser element (not shown) for emitting a spot beam modulated in accordance with the image data; a polygon mirror (deflecting device) 240 for deflecting the laser beam from the semiconductor laser element, in the main scan direction; an f-theta lens 241 for focusing the laser beam deflected by polygon mirror 240 onto the surface of photoreceptor drum 222a-222d; and mirrors 242 and 243.

The pixel signal corresponding to the black component image of a color original image is supplied to laser beam scanner unit 227a; the pixel signal corresponding to the cyan color component image of a color original image is supplied to laser beam scanner unit 227b; the pixel signal corresponding to the magenta color component image of a color original image is supplied to laser beam scanner unit 227c; and the pixel signal corresponding to the yellow color component image of a color original image is supplied to laser beam scanner unit 227d. In this arrangement, the static latent images corresponding to the color separations of the original image information are formed on photoreceptor drums 222a to 222d. Developing units 224a, 224b, 224c and 224d hold black toner, cyan color toner, magenta color toner and yellow color toner, respectively. The static latent image on photoreceptor drum 222a-222d is developed by the toner of a corresponding color. Thus, the color separations of the original image information are reproduced in image forming unit 210 as toner images of different colors.

Provided between the first image forming station Pa and paper feeding mechanism 211 is a paper-attraction charger 228, which electrifies the conveyer and transfer belt 216 surface so that paper P fed from paper feeding mechanism 211 can be conveyed without any slip or slide, whilst being reliably attracted to conveyer and transfer belt 216, from the first image forming station Pa to the fourth image forming station Pd.

## 21

An erasing device 229 is arranged approximately right above driving roller 214 located between the fourth image forming station Pd and fixing unit 217. Applied to this erasing device 229 is an alternating current for separating paper P electrostatically attracted to conveyer and transfer belt 216, from the belt.

In the thus configured digital color copier, cut-sheet type paper is used as paper P. When paper P is delivered from the paper feed cassette into the guide along the paper conveyance path of paper feeding mechanism 211, the leading edge of paper P is detected by a sensor (not shown), which outputs a detection signal, and based on the detection signal the paper is briefly stopped by a pair of registration rollers 212. Then, paper P is sent out in synchronization with image forming stations Pa to Pd, onto conveyer and transfer belt 216 that is rotating in the direction of arrow Z in FIG. 2. At this point, conveyer and transfer belt 216 has been charged in a predetermined manner by paper attraction charger 228 as stated above, so that paper P is stably fed and conveyed during its passage through all the image forming stations Pa to Pd.

In each image forming station Pa-Pd, the toner image of each color is formed so that the different color images are superimposed on the support surface of paper P which is conveyed whilst being electrostatically attracted by conveyer and transfer belt 216.

When transfer of the image formed by the fourth image forming station Pd is completed, paper P is separated by virtue of the erasing charger, continuously starting at its leading edge, from conveyer and transfer belt 216 and introduced into fixing unit 217. Finally, paper P having the toner image fixed thereon is discharged through the paper discharge port (not shown) onto paper output tray 220.

In the above description, the photoreceptors are exposed to scanning laser beams from laser beam scanner units 227a-227d, so that optical images are written onto the photoreceptors. However, instead of the laser beam scanner units, another optical writing system (LED head) made up of a light emitting diode array with a focusing lens array may be used. In this case, an LED head is smaller in size compared to the laser beam scanner unit and has no moving parts hence is silent. Therefore, this LED head can be preferably used for an image forming apparatus, such as a tandem type digital color copier, which needs multiple optical writing units.

In actual usage circumstances, such a color image forming apparatus is not only used for color printing but is often used for printing of monochrome (black and white) images. A typical operational control made in accordance with user mode selection will be described with reference to the flowchart shown in FIG. 3. First, when color image output mode is selected (Y at Step S1), all the photoreceptors 222a, 222b, 222c and 222d are set at the ordinary positions where they come in contact with conveyer and transfer belt 216 (S2). Then all the photoreceptors 222a, 222b, 222c and 222d are driven to rotate to implement charging, development and other necessary operations for each of the photoreceptors 222a, 222b, 222c and 222d, in accordance with the electro-photographic process (S3), whereby a color image is formed on a sheet of paper.

On the other hand, when black/white image output mode is selected (N at S1), a separation/abutment mechanism is actuated so that photoreceptors 222b, 222c and 222d for yellow (Y), magenta (M) and cyan (C) are separated from conveyer and transfer belt 216 (S5). Then, drives of these photoreceptors 222b, 222c and 222d are turned off to stop them rotating (S6). At the same time, charging, development and other necessary operations for these photoreceptors 222b, 222c and 222d are turned off (S7). In this condition, photoreceptor 222a for black development is driven to rotate (S8) to implement charging, development and other neces-

## 22

sary operations for the photoreceptor 222a for black development, in accordance with the electrophotographic process (S9) to thereby produce a monochrome image with black toner on a sheet of paper.

In the above way, when the black/white image output mode is selected, photoreceptors 222b, 222c and 222d, other than photoreceptor 222a for black development, are set into a non-active state by stopping the rotation or in some other way and caused to part with transfer and conveyance belt 216. Accordingly, it is possible to reduce the risk of coating abrasion of photoreceptors 222b, 222c and 222d which are unused in the black/white image output mode, due to the cleaning blades and printing paper, transfer and conveyance belt 216, etc, to as low as possible.

Such an image forming apparatus usually has a storage means, so that it is possible to know in what ratio black/white and color copy operations are implemented in the image forming apparatus, or what sizes of copies are used. Statistical analysis of these pieces of data from the market makes it possible to evaluate the setting of the durable factor of the photoreceptor for black and the photoreceptors for other development colors, which will minimize the waste of replacement. From such evaluation of data, it was found to be preferred that the photoreceptors of the present application should satisfy the following relation:

$$0.5 < (X/Y) < 0.8,$$

where X represents the reduction in film thickness ( $\text{\AA}$ ) per  $1 \times 10^7$  mm of the traveling distance of the photoreceptor for black development and Y represents the reduction in film thickness ( $\text{\AA}$ ) per  $1 \times 10^7$  mm of the traveling distance of the photoreceptors for the other development colors.

Here, when  $(X/Y)$  is greater than 0.8, or the reduction of the photoreceptor for black in film thickness per unit traveling distance is greater, and beyond the predetermined range, the photoreceptor for black development will degrade earlier than the photoreceptors for the other development colors if the machine is used more often for black/white copying operations. If the machine is used without maintenance, it cannot keep good image quality because of color imbalances. However, replacement of only the photoreceptor for black development in this situation will also cause color imbalance, resulting in failure to maintain good image quality. Replacement of all the photoreceptors results in large wastefulness because the photoreceptors for the other development colors which are still usable must also be discarded.

When  $(X/Y)$  is smaller than 0.5, the photoreceptors for the other development colors will degrade earlier than the photoreceptor for black development if the machine is used more often for color copying operations. If the machine is used without maintenance, it cannot keep good image quality because of color imbalances. However, replacement of the photoreceptors for the other development colors in this situation will also cause color imbalance, resulting in failure to maintain good image quality. Replacement of all the photoreceptors results in large wastefulness because the photoreceptor for black development which is still usable must be discarded.

In the present invention, limiting these factors to the predetermined ranges makes it possible to meet the market demands of the great majority of users. Specific methods of limiting the abrasion characteristics of the photoreceptors within the predetermined ranges in the present invention can be mentioned as follows:

1. For the binder resin for the photoreceptor for black development, a binder resin with higher resistance to abrasion than that for the photoreceptors for the other development colors may be selected.

23

2. The usage ratio of the charge transport material for the binder resin used for the photoreceptor for black development may be adjusted to be lower than that for the photoreceptors for the other development colors (the proportion of the binder resin is made higher).  
 3. A low friction material such as polyvinylidene fluoride may be added to the photoreceptor for black development. With these methods, the abrasion resistance of the photoreceptors can be adjusted. However, the present invention should not be limited to these.
- (Embodiment)

Specific examples of the present invention will be described herein-below.

### EXAMPLE 1

As a conductive substrate 1 shown in FIG. 1, an aluminum drum with 40 mm in diameter and 340 mm in length was used. Four parts by weight of titanium oxide particles and 6 parts by weight of a copolymer nylon resin (trade name: CM8000, a product of Toray Industries, Inc.) as a binder resin were added to a mixed solvent consisting of 35 parts by weight of methyl alcohol and 65 parts by weight of 1,2-dichloroethane. Then the mixed solvent was dispersed for eight hours using a paint shaker so as to prepare an undercoat layer application liquid. Then the thus obtained application liquid was charged into a tank. The aluminum drum was dipped into the liquid, forming an undercoat layer 5 of 0.9  $\mu\text{m}$  thick on the aluminum drum. Since the solvent evaporates during drying, titanium oxide particles and copolymer nylon resin remain as the undercoat layer, which consists of 40 wt % titanium oxide particles and 60 wt % binder resin.

24

0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers.

5



15 The thus prepared coating liquid for charge transport layers was dip coated over the charge generation layer formed as above. After drying for 1 hour at 120°C., a charge transport layer of about 20  $\mu\text{m}$  thick was formed. Thus, a layered photoreceptor shown in FIG. 1 was prepared as a photoreceptor for black development.

20 Similarly, 100 parts by weight of a charge transport material: the aforementioned butadiene compound (the example compound (2-2)) and 140 parts by weight of a polycarbonate resin compound having the following constitutional formula (example compound (7): a copolymer containing three types of repeat units in a 0.0001:0.85:0.1499 mol ratio) as a binder resin, 5 parts by weight of 2,6-bis-tert-butyl-4 methylphenol (Sumilizer BHT, a product of Sumitomo Chemical Co., Ltd.) as an antioxidant and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers.

25

30

35



50 Subsequently, two parts of oxo-titanyl phthalocyanine pigments at least presenting a clear peak at a Bragg angle ( $2\theta \pm 0.2^\circ$ ) of  $27.3^\circ$  by CuK $\alpha$  characteristic X-ray diffraction shown in FIG. 4, one part of a polyvinyl butyral resin (trade name: S-LEC BMS, a product of SEKISUI CHEMICAL CO., LTD.) and 97 parts of dichloroethane were dispersed for 12 hours using a ball mill dispersing machine to prepare a dispersed liquid. The thus obtained liquid was charged into a tank, and the aluminum drum with undercoat layer 5 formed thereon was dip coated to form a charge generation layer 2 of about 0.2  $\mu\text{m}$  thick over the undercoat layer.

Further, 100 parts by weight of a charge transport material: the aforementioned butadiene compound (the example compound (2-2)) and 140 parts by weight of a polycarbonate resin having the following constitutional formula (example compound (6)) as a binder resin, 5 parts by weight of 2,6-bis-tert-butyl-4 methyl phenol (Sumilizer BHT, a product of Sumitomo Chemical Co., Ltd.) as an antioxidant and

55 The thus prepared coating liquid for charge transport layers was dip coated over the charge generation layer formed as above. After drying for 1 hour at 120°C., a charge transport layer of about 20  $\mu\text{m}$  thick was formed so as to be used for the photoreceptors for color development. Here, the amount of solvent was adjusted as appropriate, taking into consideration the viscosity and coatability.

60 The thus fabricated electrophotographic photoreceptors were set on a tandem type full-color copier (a modified AR-C150 (a product of Sharp Corporation) of which drum drive and transfer belt drive were permitted to be varied arbitrarily). The image characteristics and reduction in film thickness of each photoreceptor at the initial stage and after a copying operation of 40,000 sheets, specifically, 12,000 copies of a black/white original having 10% image density (with color drums stopped and kept away from the recording sheet transfer belt) and 28,000 copies of an original having 10% image density for each of K(BK), C, M and Y, were

25

measured. In this operation, the traveling distance of the drum for black development was  $4 \times 10^7$  mm, and the traveling distance of each color drum was  $2.8 \times 10^7$  mm. The result is shown in Table 1 below.

## EXAMPLE 2

Photoreceptors were prepared and evaluated in the same manner as in example 1, except that a polycarbonate resin having the following constructional formula (example compound (8)) was used as the binder resin for the photoreceptor for black development and the aforementioned example compound (1-1) (trade name: Z-400, a product of Mitsubishi Engineering plastics Co.) was used as the polycarbonate resin for the photoreceptors for colors. The result is shown in Table 1.



## COMPARATIVE EXAMPLE 1

Photoreceptors were prepared and evaluated in the same manner as in example 1, except that the aforementioned example compound (6) (having the same composition as the polycarbonate resin used for the photoreceptor for black development) was used as the polycarbonate resin for the photoreceptors for colors. The result is shown in Table 1.

## COMPARATIVE EXAMPLE 2

Photoreceptors were prepared and evaluated in the same manner as in example 1, except that a polyacrylate resin (trade name: U-100, a product of UNITIKA LTD.) was used for the polycarbonate resin used for the photoreceptors for colors, and dichloromethane was used as the solvent instead of tetrahydrofuran. The result is shown in Table 1.

## EXAMPLE 3

The conductive substrate, undercoat layer and charge generation layer were formed in the same manner as in example 1. Then, 100 parts by weight of a charge transport material: the aforementioned example compound (2-2) and 160 parts by weight of the aforementioned copolymer resin (example compound (7)), 5 parts by weight of 2,6-bis-tert-butyl-4 methyl phenol (Sumilizer BHT, a product of Sumitomo Chemical Co., Ltd.) and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers. The thus prepared coating liquid for charge transport layers was dip coated over the charge generation layer 2 formed as above. After drying for 1 hour at 120° C., a charge transport layer 3 of about 20  $\mu\text{m}$  thick was formed. Thus, a layered photoreceptor shown in FIG. 1 was prepared as a photoreceptor for black development.

Similarly, 100 parts by weight of a charge transport material: the aforementioned example compound (2-2) and 160 parts by weight of the aforementioned copolymer resin (example compound (7)), 5 parts by weight of 2,6-bis-tert-butyl-4 methyl phenol (Sumilizer BHT, a product of Sumitomo Chemical Co., Ltd.) and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers. The thus prepared coating liquid for charge transport layers was dip coated over the charge generation layer 2 formed as above. After drying for 1 hour at 120° C., a charge transport layer 3 of about 20  $\mu\text{m}$  thick was formed. Thus, a layered photoreceptor shown in FIG. 1 was prepared as a photoreceptor for black development.

5 aforementioned polycarbonate resin (example compound (1-1), tradename: Z-400, a product of Mitsubishi Engineering plastics Co.), 5 parts by weight of 2,6-bis-tert-butyl-4 methyl phenol (Sumilizer BHT, a product of Sumitomo Chemical Co., Ltd.) and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers. The thus prepared coating liquid for charge transport layers was dip coated over the charge generation layer 2 formed as above. After drying for 1 hour at 120° C., a charge transport layer 3 of about 20  $\mu\text{m}$  thick was formed so as to be used for the photoreceptors for color development. Here, the amount of solvent was adjusted as appropriate, taking into consideration the viscosity and 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 981

## COMPARATIVE EXAMPLE 3

Photoreceptors were prepared and evaluated in the same manner as in example 3, except that a commercially available bisphenol-A polycarbonate (trade name: C-1400, a product of TEIJIN CO., LTD.) was used for both the polycarbonate resins for black and colors. The result is shown in Table 1.

## COMPARATIVE EXAMPLE 4

Photoreceptors were prepared and evaluated in the same manner as in example 3, except that the drums for colors were neither stopped nor kept away from the recording sheet conveyer belt during the black and white image output mode. In this case, the traveling distances of the drums for black and colors were  $4 \times 10^7$  mm. The result is shown in Table 1.

## EXAMPLE 7

The conductive substrate, undercoat layer and charge generation layer were formed in the same manner as in example 1.

Then, 100 parts by weight of a charge transport material: the aforementioned example compound (2-2), 80 parts by weight of the aforementioned copolymer resin: the polycarbonate resin shown as example compound (6), 80 parts by weight of the aforementioned polycarbonate resin shown as example compound (1-1) (trade name: Z-200, a product of Mitsubishi Engineering plastics Co.), 5 parts by weight of 2,6-bis-tert-butyl-4 methyl phenol (Sumilizer BHT, a product of Sumitomo Chemical Co., Ltd.) and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers. The thus prepared coating liquid for charge transport layers was dip coated over the charge generation layer formed as above. After drying for 1 hour at 120° C., a charge transport layer of about 27  $\mu\text{m}$  thick was formed. Thus, a layered photoreceptor shown in FIG. 1 was prepared so as to be used for the photoreceptor for black development.

Similarly, 100 parts by weight of a charge transport material: the aforementioned example compound (2-2), 80 parts by weight of the aforementioned copolymer resin: the polycarbonate resin shown as example compound (7), 80 parts by weight of the aforementioned polycarbonate resin shown as example compound (1-1) (trade name: Z-200, a product of Mitsubishi Engineering plastics Co.), 5 parts by weight of 2,6-bis-tert-butyl-4 methyl phenol (Sumilizer BHT, a product of Sumitomo Chemical Co., Ltd.) and 0.0001 part by weight of a silicone leveling agent (trade name: KF-96, a product of Shin-Etsu Chemical Co., Ltd.) were blended into 1200 parts by weight of tetrahydrofuran so as to prepare a coating liquid for charge transport layers. The thus prepared coating liquid for charge transport layers was dip coated over the charge generation layer formed as above. After drying for 1 hour at 120° C., a charge transport layer of about 27  $\mu\text{m}$  thick was formed. Thus, a layered photoreceptor shown in FIG. 1 was prepared so as to be used for the photoreceptors for color development. Here, the amount of solvent was adjusted as appropriate, taking into consideration the viscosity and coatability. The same evaluation as in example 1 was carried out. The result is shown in Table 1.

## EXAMPLE 8

Photoreceptors were prepared and evaluated in the same manner as in example 7, except that the thickness of the charge transport layer was changed to 23  $\mu\text{m}$ . The result is shown in Table 1.

## EXAMPLE 9

Photoreceptors were prepared and evaluated in the same manner as in example 7, except that the thickness of the charge transport layer was changed to 18  $\mu\text{m}$ . The result is shown in Table 1.

## REFERENCE EXAMPLE 1

Photoreceptors were prepared and evaluated in the same manner as in example 7, except that the thickness of the charge transport layer was changed to 32  $\mu\text{m}$ . The result is shown in Table 1.

## REFERENCE EXAMPLE 2

Photoreceptors were prepared and evaluated in the same manner as in example 7, except that the thickness of the charge transport layer was changed to 16  $\mu\text{m}$ . The result is shown in Table 1.

TABLE 1

|        | Film loss of BK drum ( $\mu\text{m}$ ) | Film loss of Color drums (average $\mu\text{m}$ ) | X (Å) | Y (Å) | X/Y  | Image of BK drum after 40 K prints | Image of color after 40 K prints |
|--------|----------------------------------------|---------------------------------------------------|-------|-------|------|------------------------------------|----------------------------------|
| Ex. 1  | -7.7                                   | -7.5                                              | 183   | 268   | 0.68 | Good                               | Good                             |
| Ex. 2  | -8.1                                   | -7.9                                              | 203   | 282   | 0.72 | Good                               | Good                             |
| Ex. 3  | -6.2                                   | -6.3                                              | 155   | 225   | 0.69 | Good                               | Good                             |
| Ex. 4  | -8.8                                   | -9.5                                              | 220   | 339   | 0.65 | Good                               | Good                             |
| Ex. 5  | -8.0                                   | -8.7                                              | 200   | 311   | 0.64 | Good                               | Good                             |
| Ex. 6  | -8.8                                   | -10.4                                             | 220   | 371   | 0.59 | Good                               | Good                             |
| Ex. 7  | -7.0                                   | -7.0                                              | 170   | 250   | 0.68 | Good                               | Good                             |
| Ex. 8  | -7.0                                   | -7.1                                              | 170   | 254   | 0.67 | Good                               | Good                             |
| Ex. 9  | -7.0                                   | -7.0                                              | 170   | 250   | 0.68 | Good                               | Good                             |
| Comp.  | -7.3                                   | -5.0                                              | 183   | 179   | 1.02 | Imbalance in color                 | Imbalance in color               |
| Ex. 1  | -7.3                                   | -10.9                                             | 183   | 389   | 0.47 | Imbalance in color                 | Imbalance in color               |
| Comp.  | -13.5                                  | -10.4                                             | 338   | 371   | 0.91 | Fog, white stripes                 | Fog                              |
| Ex. 3  | -6.2                                   | -9.0                                              | 155   | 225   | 1.00 | Good                               | Filming                          |
| Comp.  | -7.5                                   | -7.7                                              | 188   | 275   | 0.68 | Image blur                         | Image blur                       |
| Refer. | -7.5                                   | -7.5                                              | 188   | 268   | 0.70 | Low image, density, fog            | Low image, density, fog          |
| Ex. 1  |                                        |                                                   |       |       |      |                                    |                                  |
| Refer. |                                        |                                                   |       |       |      |                                    |                                  |
| Ex. 2  |                                        |                                                   |       |       |      |                                    |                                  |

Concerning the samples of comparative examples 1 and 2, a large difference in the reduced amount of film thickness between the drum for black development and the drums for color development occurred and the color balance after a 40K run degraded compared to the initial image. Also, it was impossible to match the end of life of all the four photoreceptors. With concern to the sample of comparative example 3, a marked reduction in film thickness occurred and image fog was observed after 25K prints. White stripes due to uneven reduction in film thickness, possibly caused by paper particles, occurred. As to the sample of comparative example 4, filming occurred on the color drums and image defects occurred with white and black stripes.

Since Reference examples 1 and 2 are a little infirm to the afore mentioned Examples, the preferable range of thickness of the photoreceptor layer is from 18 to 27  $\mu\text{m}$  as shown in Reference Examples 1 and 2.

As to the sample of Reference example 5, serious image blur occurred from the beginning of the operation, resulting in markedly poor reproducibility of dots and lines.

Concerning to the sample of Reference example 6, no problems occurred at the initial stage. However, the charging

29

characteristics became bad after 30K prints, causing density decrease and background fog.

Thus, in the present invention, differentiation of abrasion resistance between the photoreceptors for black development and for color development and limitation of the reduced amounts of the film thickness of the photoreceptive layer per unit traveling distance to the predetermined ranges make it possible to provide photoreceptors that satisfy both the durability and the electrophotographic performance. It is also possible to use all the photoreceptors and toners, for, and within, a concurrent period, and hence provide a low-cost color image forming apparatus.

In the present invention, since the photoreceptors for black and for colors are made to differ in the abrasion resistance and since the reduced amounts of the film thickness per unit traveling distance are designated to fall within the predetermined ranges, it is possible to use the drums for black and for color development for approximately the same period, without reaching a situation in which the drum for black development alone has been worn away and become unusable at an earlier time, or that the drum for black development alone has a long life because of marked abrasion resistance. Therefore, all the photoreceptors can be replaced at the same time, and it is possible to provide a low-cost color image forming apparatus.

What is claimed is:

1. A color image forming apparatus comprising a multiple number of electrophotographic image forming stations for multiple development colors including black, arranged in line in the paper feed direction, each image forming station having a photoreceptor, a charger, an exposure device, a developing device, a transfer device and a cleaning device, characterized in that the photoreceptors satisfy the following relation:

$$0.5 < (X/Y) < 0.8,$$

where X represents the reduction in film thickness (Å) per  $1 \times 10^7$  mm of the traveling distance of the photoreceptor for black development and Y represents the reduction in film thickness (Å) per  $1 \times 10^7$  mm of the traveling distance of the photoreceptors for the other development colors, and wherein the composition of the binder resin used in the photoreceptor for black development is different from one of the photoreceptors for the other development colors.

2. The color image forming apparatus according to claim 1, wherein the binder resin used for either the photoreceptor for black development or at least one of the photoreceptors for the other development colors employs a polycarbonate polymer having, at least, one structural unit represented by the following general formula (1):

30



(wherein  $R^1$ ,  $R^2$ ,  $R^3$ ,  $R^4$ ,  $R^5$ ,  $R^6$ ,  $R^7$  and  $R^8$  individually represent a hydrogen atom, halogen atom, substituted or unsubstituted alkyl of 1 to 6 carbon atoms,  $C_4$ – $C_{10}$  cyclic hydrocarbon residual group, substituted or unsubstituted aryl, and Z represents a group of atoms required to constitute a substituted or unsubstituted carbocycle or substituted or unsubstituted heterocycle, m being an integer).

3. The color image forming apparatus according to claim 2, wherein the binder resin used for either the photoreceptor for black development or the photoreceptors for the other development colors employs a polycarbonate polymer having, at least, one structural unit represented by the general formula (1).

4. The color image forming apparatus according to claim 1, wherein the photoreceptors other than that for black development are stopped operating in monochrome (black and white) copy mode.

5. The color image forming apparatus according to claim 2, wherein the photoreceptors other than that for black development are stopped operating in monochrome (black and white) copy mode.

6. The color image forming apparatus according to claim 1, wherein the photoreceptors other than that for black development are separated from the paper feed line, in monochrome (black and white) copy mode.

7. The color image forming apparatus according to claim 2, wherein the photoreceptors other than that for black development are separated from the recording media conveyor belt, in monochrome (black and white) copy mode.

8. The color image forming apparatus according to claim 1, wherein the film thickness of the photoreceptor layer ranges from 18  $\mu\text{m}$  to 27  $\mu\text{m}$ .

9. The color image forming apparatus according to claim 2, wherein the film thickness of the photoreceptor layer ranges from 18  $\mu\text{m}$  to 27  $\mu\text{m}$ .

10. The color image forming apparatus according to claim 4, wherein the film thickness of the photoreceptor layer ranges from 18  $\mu\text{m}$  to 27  $\mu\text{m}$ .

11. The color image forming apparatus according to claim 5, wherein the film thickness of the photoreceptor layer ranges from 18  $\mu\text{m}$  to 27  $\mu\text{m}$ .

12. The color image forming apparatus according to any one of claims 1 through 11, wherein the shape and/or appearance of the photoreceptor for black development or its part is made different from the shape and/or appearance of the photoreceptors or their parts for the other development colors.

\* \* \* \* \*